

March 25, 1958

R. W. HEIGES ET AL

2,828,219

FLOOR AND WALL COVERING

Filed July 29, 1955



INVENTOR  
RUSSELL W. HEIGES  
WILLIAM R. REED

*by  
Walter + Company*  
ATTORNEY

1

2,828,219

## FLOOR AND WALL COVERING

Russell W. Heiges, and William R. Reed, Pittsburgh, Pa., assignors to Armstrong Cork Company, Lancaster, Pa., a corporation of Pennsylvania

Application July 29, 1955, Serial No. 525,400

2 Claims. (Cl. 117—72)

This invention relates to a floor and wall tile having applied thereto a soil-resistant, wear-resistant coating. More particularly, this invention relates to an irregular floor and wall tile such as cork tile having applied thereto a polyethylene type protective coating to render the surface resistant to dirt and wear.

In coating floor and wall tile, such as cork tile, with a wear-resistant coating composition, it has been necessary to select a composition which will fill all of the small imperfections in the surface of the tile which are common to products formed from natural cork. In order to satisfactorily fill all of these imperfections, it has been necessary that the coating composition have a low viscosity. As a general rule, compositions having low viscosity, even though they satisfactorily fill the imperfections in the surface of the tile, do not have the wear resistance and soil resistance necessary to serve as a satisfactory coating composition. In order to overcome this difficulty, finishes have been prepared from blends of well-known waxes and polyethylene to form a coating composition with low melt viscosity and good wear and soil resistance. However, the polyethylene is not completely compatible with the wax constituents, resulting in a composition which has the disadvantage of showing white scratches on the surface under normal traffic. These scratches are difficult to remove. Crystallization of the wax also contributes to the white scratching condition.

In order to overcome the disadvantages of the prior art compositions, the present invention has been developed in which the coating is applied in a plurality of layers. The first layer is a coating composition having a low viscosity which will satisfactorily fill all of the imperfections appearing on the surface of the cork tile, and the other layer or layers are a low viscosity polyethylene type which renders the surface wear-resistant and soil-resistant. Inasmuch as the top layer or film is all of the same composition, the problem of incompatibility is not present and the white scratch marks do not occur. Polyethylene is of such nature that the problem of crystallization does not occur.

In preparing the low viscosity coating composition for the first coating, the following formulation has been found satisfactory and is presented here by way of example.

### Parts by weight

|                                                                                      |     |
|--------------------------------------------------------------------------------------|-----|
| Microcrystalline wax, melting point 190° F. to 195° F.                               | 71½ |
| Paraffin, 125° F.                                                                    | 20  |
| High molecular weight polyethylene (molecular weight of 10,000 or higher)            | 7   |
| Low molecular weight polyethylene (molecular weight ranging between 1,000 and 3,000) | 1½  |

2

It should be understood that the above is given merely as an example of the type of coating that is suitable as a first or cover coat; however, any of the low melt viscosity products can be used satisfactorily for this purpose.

5 The above coating composition is applied as a hot melt application at a regular two-roll coating device. The coating composition forms a pool between the applicator roll and a second roll. The sheet of material to which the hot melt is to be applied is passed between the applicator roll and a back-up roll in such manner that the film of wax adhering to the applicator roll is transferred therefrom onto the surface of the sheet of material passing through the device. The sheet then passes through an ironing roll heated to a temperature of approximately 380° F., which irons the coating composition firmly onto the surface of the tile and smooths out any ridges or grapevining appearing on the surface. This forms a tile having a relatively smooth coating applied thereto, filling all of the small imperfections in the surface of the cork tile.

10 20 The drawing illustrates a piece of cork tile 2 comprised of compressed cork particles 3. To this cork tile sheet there is applied a dual coating of wax in which the first layer 4 applied directly to the surface of the cork particles 3 is a blend containing a major portion of hydrocarbon wax and a minor portion of a polyethylene polymer having a relatively high molecular weight, and the surface coating 5 is a polyethylene polymer having a relatively low molecular weight.

25 The top or wear coating comprises a film of polyethylene of a relatively low molecular weight ranging between 1,000 to 3,000. This coating of polyethylene is applied from a hot melt of the polyethylene placed in the two-roll applicator in the same manner as expressed for the first coating. The polyethylene coating is also ironed onto the surface. The system outlined above results in a cork tile having a relatively low viscosity first coat which fills all the imperfections and which has applied thereover a coat of a relatively hard polyethylene wax, forming a smooth wear- and soil-resistant surface

30 40 45 50 55

on the product.

The invention may be carried out by substituting a 100% polyethylene coating for the first coating to be applied to the cork tile. When using this modification, it is recommended that a polyethylene material of a relatively low molecular weight, such as that falling within the range of 1,000 to 3,000, be used to cover the imperfections in the tile. This first coating of polyethylene should be rather thin so as to flow into the imperfections. This coating is ironed onto the surface of the cork tile in the same manner as described earlier. The additional second coat of polyethylene is then applied thereover in the manner expressed above. Either of the systems outlined herein produces a finish which is relatively hard, wear-resistant, and soil-resistant, and has the high gloss desirable in a product of this type.

60 65 It will be obvious from the foregoing that we have developed a floor and wall covering having applied thereto a finish which adequately fills all the imperfections in the surface of the tile and presents a smooth hard glossy wear- and soil-resistant surface which is easy to maintain.

We claim:

1. A cork composition floor and wall covering having a wear-resistant finish comprising a film of a blend containing a major portion of hydrocarbon wax and a minor portion of a polyethylene polymer having a molecular

weight in excess of 10,000 and a surface coating of a polyethylene polymer having a relatively low molecular weight falling within the range of 1,000 to 3,000.

2. A cork composition floor and wall covering having a wear-resistant finish comprising a film of a blend containing about 70% of hydrocarbon wax and about 7% of a polyethylene polymer having a molecular weight in excess of 10,000 and a surface coating of a polyethylene polymer having a relatively low molecular weight falling within the range of 1,000 to 3,000. 5

10

## References Cited in the file of this patent

## UNITED STATES PATENTS

- |           |              |                |
|-----------|--------------|----------------|
| 1,824,885 | Hammond      | Sept. 29, 1931 |
| 2,290,794 | Alvarado     | July 21, 1942  |
| 2,698,309 | Clark et al. | Dec. 28, 1954  |

## FOREIGN PATENTS

- |         |               |               |
|---------|---------------|---------------|
| 566,745 | Great Britain | Jan. 11, 1945 |
|---------|---------------|---------------|